

1

3,836,468

**GREASES THICKENED WITH KETO FATTY ACID LITHIUM SOAPS OR KETO CYANOETHYLATED FATTY ACID LITHIUM SOAPS**

Harold E. Kenney, Jenkintown, Edward T. Donahue, Philadelphia, and Gerhard Maerker, Orelan, Pa., assignors to the United States of America as represented by the Secretary of Agriculture

No Drawing. Original application July 25, 1972, Ser. No. 275,010. Divided and this application Aug. 24, 1973, Ser. No. 391,183

Int. Cl. C10m 5/14, 5/20, 7/30

U.S. Cl. 252—33.6

5 Claims

**ABSTRACT OF THE DISCLOSURE**

Keto fatty acids or derivatives of keto fatty acids are cyanoethylated and the resulting three carbon cyanoethyl branched chain fatty acids are mixed with an appropriate amount of a diester or a petroleum base oil. The mixture is then reacted in situ with a dilute aqueous solution of lithium hydroxide to obtain a stable grease.

This is a division of application Ser. No. 275,010, filed July 25, 1972.

A non-exclusive, irrevocable, royalty-free license in the invention herein described, throughout the world for all purposes of the United States Government, with the power to grant sublicenses for such purposes, is hereby granted to the Government of the United States of America.

This invention relates to lithium polycyanoethylated keto fatty soaps and more specifically to the use of such soaps to make multipurpose greases.

Small amounts of certain chemical compounds are commonly added to lubricants to improve their physical properties. Typical additives include oxidation or corrosion inhibitors, wear improvers, water repellents, and dyes. One problem in formulated greases containing additives is that in storage and in use these additives tend to migrate in the base oil and in extreme cases cause the grease to separate. Another problem is the frequent tendency for two additives to be incompatible which complicates the task of formulation.

Most lubricants are blended with an additive to improve their anti-wear function. The soaps of this invention improve the wear properties of the base oils with which they are mixed without use of additives. Another important feature of this invention is that the functional groups responsible for anti-wear and grease forming properties are incorporated into the same molecule. Consequently, it is impossible for migration or incompatibility to occur in greases made from these soaps.

The polyfunctional fatty soaps of this invention form two classes of stable greases, one based on diester type oils, the other on petroleum oils. The diester based greases have good anti-wear properties and better than average thermal stability while the petroleum based greases have good thermal stability and better than average anti-wear properties.

An object of this invention is to prepare stable greases by dispersing polyfunctional soaps in synthetic base oils of the diester type.

Another object of this invention is to prepare stable greases by dispersing polyfunctional soaps in petroleum oil of lubricating viscosity such as 100 paraffin oil.

Still another object is to provide polyfunctional fatty soap derivatives that impart thermal stability and anti-wear properties to greases.

In general, according to this invention the above objects are accomplished by dispersing in petroleum oil or in a

2

synthetic oil of the diester type, a polyfunctional fatty soap of the general formula.



wherein the sum of  $x$  and  $y$  is a number from 5 to 17 and  $\text{R}$ ,  $\text{R}^1$ ,  $\text{R}^2$ , and  $\text{R}^3$  are hydrogen or  $-(\text{CH}_2)_2\text{C}\equiv\text{N}$ .

As seen in the formula above, these fatty derivatives are novel compounds in which from 1 to 4 three carbon side chains having a terminal nitrile groups are attached to the carbons and to the ketone.

Suitable starting materials for the greases formed in this invention are keto fatty acids or their derivatives either naturally occurring or synthesized by suitable known procedures. The keto fatty derivative is dissolved in an excess of acrylonitrile containing a small amount of water to inhibit polymerization. Addition of a catalytic amount of strong base to this mixture causes the formation of products in which from one to four  $\beta$ -cyanoethyl groups are attached to the carbon atoms which are adjacent to the ketone group. The product mixture is recovered after acidification of the reaction mass.

The unreacted fatty ketone is recovered by extracting the reaction mixture with hexane. The  $\beta$ -cyanoethyl branched fatty acids are then mixed with the appropriate amount of the desired base oil. The mixture is then treated in situ with a dilute aqueous solution of lithium hydroxide. It was found desirable to add about 2% of an emulsifier, sorbitan monooleate. The mixture is stirred to 110° C. until the proper degree of dehydration is obtained to yield a stable grease with the desired consistency. The degree of cyanoethylation of the keto fatty acid will vary depending on conditions such as temperature and concentration of reactants. For the purposes of this invention, conditions were chosen to give an average of two cyanoethyl groups per molecule.

The diester based greases formed from this lithium polycyanoethylated fatty soap show considerably better anti-wear properties and somewhat better thermal stability than a diester based grease prepared from sodium stearate. The petroleum based greases formed from this fatty soap derivative have improved anti-wear properties and much better thermal stability than a standard sodium stearate petroleum based grease.

In the preparation of the cyanoethyl fatty grease precursor, suitable keto fatty acids may vary in chain length from 10–22 carbon atoms with the carbonyl group attached at any point on the chain.

The diester based greases can be formulated using any of the common commercial diester oils such as di(2-ethylhexyl) sebacate (D.O.S.). Suitable oils for the petroleum based greases may be any hydrocarbon oil of lubricating viscosity such as 100 paraffin oil.

The amount of polycyanoethyl fatty soap used in this invention to form greases is generally less than 20% by weight of formulated grease.

It is important that the grease formed is not overheated or the small amount of water necessary for the oil, water, soap complex will be driven off causing the soap to precipitate.

The ureacted keto fatty acid can be recovered or may be left in the reaction mixture. Its presence does not affect the grease forming properties but does reduce the beneficial effects on wear and thermal properties.

The thermal stability properties of the greases described in this patent were determined using the dropping point method (ASTM D-566). This procedure measures the temperature at which the grease passes from a semi-solid to a liquid state and is a qualitative indication of the heat resistance of the grease.

Anti-wear properties were determined using the Shell Four Ball Wear Tester as described by ASTM designation D2266-64T. Federal test method standard No. 7916. Approximately 10 ml. of the grease to be tested is placed in the test cup so that the three bottom stationary balls are covered. After positioning the cup on its stand in contact with the fourth ball, the grease was heated to 75° C., a 40 kg. load was placed on the weight tray, and the upper ball was allowed to rotate at 1200 r.p.m. for 1 hour. The diameters of the scars worn on the three stationary balls were measured by means of a low power microscope. The hardness of the greases was determined with a Penetrometer as described by ASTM designation D217-48. A microcone was used to check the consistency of small samples.

The invention is illustrated by the following examples.

#### EXAMPLE 1

50 g. (0.186 moles) of methyl 12-ketostearate was dissolved in 336 g. (6.3 moles) of acrylonitrile containing 8 ml. water. To this mixture was added with stirring, 24 ml. of a 40% aqueous solution of benzyltrimethylammonium hydroxide. The mixture was allowed to stir for 1 hour and then diluted with 300 ml. of water and 200 ml. of acetone. The mixture was then acidified with HCl and extracted with three 400 ml. portions of ether. The combined extracts were washed with water, dried over sodium sulfate and evaporated to a residue weight of 68.4 g. Gas-liquid chromatography (GLC), thin layer chromatography (TLC), and infrared (IR) analysis confirmed that the residue was predominately a mixture of mono, di, tri and tetra cyanoethylated ketostearate isomers plus some unreacted ketostearate. Recrystallization from hexane removed the unreacted ketostearate. GLC and elemental analysis showed the recrystallized product averaged about two cyanoethyl groups per molecule.

#### Preparation of Diester Grease

To a vigorously stirred mixture of 8.5 g. di(2-ethylhexyl) sebacate (D.O.S.), 1.5 g. cyanoethylated 12-ketostearic acid, 0.2 g. sorbitan monooleate and 1 ml. water at 110° C. was added a dilute solution of lithium hydroxide until the acid was neutralized. Stirring and heating at 110° C. was continued until the mixture began to thicken. It was then allowed to cool to room temperature with stirring. A stable grease of grade 1 hardness formed having an average wear scar of 0.564 mm. and a dropping point of 379° F.

#### Preparation of Petroleum Grease

Using the above procedure but substituting 8.5 g. of 100 paraffin oil for the base oil, the cyanoethylated 12-ketostearic acid gave a stable grease of grade 1 hardness having an average wear scar of 0.715 mm. and a dropping point of 383° F.

#### EXAMPLE 2

5.3 g. (0.018 moles) of 9(10) ketostearic acid was treated with benzyltrimethylammonium hydroxide in a 40% methanol solution until a pH of 10 was reached. The methanol was driven off with heat, and the soap product was dissolved in 5 ml. pyridine, 1 ml. water and

5 50 ml. acrylonitrile (0.75 moles). To this mixture was added slowly with stirring 2.5 ml. of a 38.5% aqueous solution of benzyltrimethylammonium hydroxide. After a half hour of stirring the reaction was diluted with 20 ml. H<sub>2</sub>O and 10 ml. acetone and then HCl was added until a pH of 2 was reached. The resulting mixture was extracted with three 50 ml. portions of ether. The combined extracts were washed with water, dried over sodium sulfate and evaporated to a residue weight of 6.4 g. GLC analysis confirmed that the residue was predominantly a mixture of mono, di, tri and tetra cyanoethylated ketostearate isomers plus some unreacted ketostearic acid. Recrystallization from a benzene ether mixture removed the unreacted material.

10 15 Preparation of Diester Grease

In a manner similar to that of Example 1, a diester grease was prepared from the cyanoethylated 9(10) ketostearic acid. This product formed a stable grease of grade 0 hardness having an average wear scar of 0.524 mm. and a dropping point of 339° F.

#### Preparation of Petroleum Grease

A 100 paraffin oil grease was prepared as in Example 1. This 100 paraffin oil based grease formed from the cyanoethylated 9(10) ketostearic acid gave a stable grease of grade 1 hardness having an average wear scar of 0.677 mm. and a dropping point of 358° F.

Attempts were made to substitute sodium, calcium, and aluminum in place of lithium but only negative results were obtained. Greases could not be made with these substitutes.

We claim:

1. A multipurpose grease comprising a major amount of lubricating oil selected from the group consisting of paraffin oil and aliphatic diester oil and a minor thickening amount of a lithium soap of the general formula



wherein the sum of x and y is a number from 5 to 17 and R, R<sup>1</sup>, R<sup>2</sup>, and R<sup>3</sup> are selected from the group consisting of hydrogen and -(CH<sub>2</sub>)<sub>2</sub>-C≡N.

2. The grease of Claim 1 wherein the lubricating oil is paraffin oil.

3. The grease of Claim 2 wherein the sum of x and y is 13.

4. The grease of Claim 1 wherein the lubricating oil is di(2-ethylhexyl) sebacate.

5. The grease of Claim 4 wherein the sum of x and y is 13.

#### References Cited

#### UNITED STATES PATENTS

3,009,878 11/1961 Eckert ----- 252-41  
3,278,431 10/1966 Morway et al. ----- 252-39

DANIEL E. WYMAN, Primary Examiner

I. VAUGHN, Assistant Examiner

U.S. Cl. X.R.

252-41, 400